

Jan. 19, 1926.

1,570,504

L. LANE

ROOF OR BUILDING TILE

Original Filed March 4, 1924

Fig. 1,



Fig. 2,



Fig. 3.



WITNESSES

Edw Thorpe  
J. L. McAniff

INVENTOR

Louis Lane  
BY Munn & Co  
ATTORNEYS

Patented Jan. 19, 1926.

1,570,504

# UNITED STATES PATENT OFFICE.

LOUIS LANE, OF HABANA, CUBA.

## ROOF OR BUILDING TILE.

Application filed March 4, 1924, Serial No. 696,851. Renewed December 12, 1925.

To all whom it may concern:

Be it known that I, LOUIS LANE, a citizen of the United States of America, and a resident of Habana, Cuba, have invented a new and Improved Roof or Building Tile, of which the following is a description.

My invention relates to a novel roofing or building element having any one of the non-ferrous metals, such as aluminum, nickel, copper, zinc, lead, etc., or their alloys and employed in the form of a very thin sheet, or foil-form as an outer protection cover or surfacing on a body of cast or moulded plastic material, or materials, such, for example, as clay, cement, asbestos or asbestos-cement, magnesite, etc., by the use of an adhesive asphaltic cementing substance between said foil-metal covering and said body.

20 The protected elements may be in any approved form of tiles, shingles, or flat or corrugated or other sheets, etc.

By the use of the non-ferrous foil-metal covering cemented on by an asphaltic adhesive material to the body mentioned, I secure all the advantages of non-ferrous metal surfaced roof with a minimum amount of metal. At the same time certain defects inherent in the roofing elements 30 generally used are eliminated and all the useful qualities for which such elements are employed are retained and conserved through the protection afforded to them by the said non-ferrous foil-metal covering and 35 by the asphaltic cementing medium used in uniting them together. The strength of the foil-metal and that of the asphaltic cement is united with the strength of the roofing or other element employed thus greatly increasing also its strength, its durability and the weathering qualities to a marked extent, and at a relatively small cost.

Reference is to be had to the accompanying drawings forming a part of this specification, it being understood that the drawings are merely illustrative of practical examples of the invention.

Figure 1 is a cross section of an arched tile formed in accordance with my invention;

Figure 2 is a longitudinal vertical section as indicated by the line 2-2 of Figure 1;

Figure 3 is a view similar to Figure 1 but showing the embodiment of the invention in a corrugated tile.

To secure the objects of my invention I employ any moulded or cast plastic material roofing elements in common use for the body portion 10 (Figs. 1 and 2) of my improved roofing and apply thereto a coating 11 of asphaltic adhesive material over which is applied a protective covering 12 of non-ferrous metal in a thin layer or foil form to cover all of the exposed surfaces of the body, including all weathering edges and the overlapping of the metal coating on to the under side of said body element sufficiently far to securely attach said foil-metal. The mentioned foil-metal covering may be and preferably is of such thickness as to afford a durable surface protection but materially thinner than the metal roof covering as used generally by itself.

In the corrugated form of tile as in Figure 2 the same features are embodied, there being a body 110 corresponding with the body 10, a coating 111 of asphaltic material as referred to and a non-ferrous foil-metal protective covering 112. In both examples it will be noted that the asphaltic coating and the protective covering are extended about the under surface adjacent the end edges so that all exposed surfaces are protected.

The thickness of the foil-metal employed will vary with the kind of metal or alloy used to make it, but it is preferably not less than 0.001 of an inch thick, nor more than 0.01 of an inch thick; and the term foil-metal as herein used is understood to cover such thicknesses although it is not to be understood as precluding the use of a somewhat thinner or thicker foil if found desirable in some metals. In practice the foil-metal covering, cut to proper size and form is coated on its seating surface when at about 300° Fahrenheit with the plastic asphaltic-cement compound which may be directly applied thereto or applied upon a previously applied primer, using for the primer some suitable vegetable oil such as linseed or Chinawood oil that has been properly heat treated before applying. The body 10 is also heated to a temperature of at least 100° Fahrenheit above the melting point of the asphaltic-cement compound which preferably should have a fusing point of not less than 250° Fahrenheit and the melted compound is applied in any suitable way to the surface of the body to be

metal protected using the minimum amount of compound therefor that may be sufficient to seal the porosity of the surface of the said body and to form a practically smooth seating surface thereon to receive the foil-metal protection. Immediately after being coated and while still at a temperature near to fusion, the previously coated foil-metal covering is applied to the body 10 and 5 pressed or rolled firmly and uniformly by any suitable means on to the said asphalt covered surfaces of the body.

With certain metals and alloys the priming of the attaching metal surface may be 10 omitted and with some metals the asphaltic coating of the attaching metal surface may also be dispensed with and the metal may be applied directly to the asphalted surface 15 of the body element as described.

20 The foil-metal may be given such surface form treatment while still hot as may be desired. It will also be apparent that, when cold any color treatment of the foil-metal surface desired may be produced 25 thereon by oxidizing or other suitable processes.

It may be stated that most plastic material roofing elements have whether cast, moulded, or pressed to shape certain common 30 defects in varying degree.

Among these defects may be mentioned, for instance, the relative softness and porosity of most common clay and cement and asbestos-cement roofing tiles, etc., that results 35 in an unpleasing surface texture and color and causes such tiles, etc., to absorb an excessive amount of rain water thereby causing an excessive loading of the roof structure as well as the deterioration and softening 40 of the tile itself. This causes also in northern climates, frost breakage, and in hot damp tropic like climates ugly discolorations from the vegetable or fungoid growths that establish themselves on such water soaked moist surfaces and blacken 45 them.

Similarly like defects exist in corrugated or other sheets made of cement and various 50 compounds of cement with asbestos, and of magnesite compounds, etc. The tendencies to further weathering and decay inherent in low grade asbestos products, used as roofing and exposed to the weather 55 may be mentioned also as a further serious defect to be overcome in asbestos-cement elements.

60 This defect of softness and porosity and consequent great absorption pertaining to the softer clay and other cast or plastic made roofing elements mentioned as well as their consequent lack of good weathering properties, is corrected and overcome by the well-known water-proofing quality of the asphaltic saturating cement employed by me, 65 which being applied in a fused state to the

higher heated surface of the tile or other element enters into and effectively seals the treated surface against all absorption and moisture and at the same time gives a 70 smooth and adherent medium for cementing thereto the protecting foil-metal covering which in turn acts to conserve and protect the asphaltic compound employed as a cementing medium from all changes of 75 oxidation and deterioration; the two together at the same time adding to the protected element a very material increased factor of safety against breakage in handling, shipping, installing and when installed on the roof, over that of the unprotected tile 80 or other elements, this attribute constituting an important and useful feature of my invention.

Properly refined bitumens or asphalts and 85 allied substances, such as I employ in my cementing compound have well known weather resisting properties but are subject to gradual changes brought about by oxidation or condensation through exposure to air, light, heat and gases. But when such 90 asphaltic materials are used as I employ them protected by the metal covering from light and air and gases and exposed normally to medium temperature relative to 95 their fusing points such asphaltic compounds have an almost unmeasured durability fully commensurate with the other components employed in my roofing element, so that by the processes employed and by the manner of my combining together 100 the materials stated there is brought about complementary important improvements and economies over the present methods now in use as to such materials for the purposes stated and whereby the use of such materials for roofing purposes and otherwise will 105 be greatly extended.

It may be asserted that the non-ferrous metals constitute the most perfect, most durable and most beautiful roof surfacing materials in use; and that the use of such metals is limited by several considerations such as the great expense owing to the necessity of the relatively great thickness of 110 such metals when used as at present in order to give stiffness and strength by themselves which makes a roof of such metals as at present made of too great cost. It will be observed that the thickness of the non-ferrous metals, as at present used alone in the 115 sheet form for roofing material, bears no relation to the requirements as to durability, considered from the standpoint of weather resistance, or for protection against the element; but is determined solely by structural 120 considerations thus another important feature arising from my improved method of employment of such non-ferrous metals in their foil form is the consequent extended 125 use of such metals brought about through 130

the very great economy secured by their use in said foil-form as stated.

Another consideration limiting the use for roofing purposes of such metals in ordinary sheet form is their relatively high conductivity of heat and cold and the consequent lack of protection afforded to the building against the temperature changes to which it is exposed. For this reason roofs of such metals are scarcely ever employed in very hot countries, and their use is made very limited in cold countries owing to the expensive underwork needed to supply this temperature protection by independent means.

Besides when tiles, shingles, etc., as now made in such metals in hollow sheet metal form are used, they become merely metallic imitations of the plastic roof forms and the obviousness of this lack of solidity is a detriment to their use; whereas in the improved method employed in my invention such metals used in the foil-form combined with the solid body elements stated are accepted as a surface protective treatment of the solid body forms in the same way as a glazing is considered on clay tile and the objection referred to is overcome.

I am aware of the over all coating of surfaces of ferrous roofing metal elements with asphaltic preparations to protect them from corrosion and electrolysis, etc., and of the use of asbestos and other materials to cover over and protect the asphaltic coating thus employed, as well as of the use of sand, pebbles, crushed stone and other coatings and surfacings for that purpose over asphaltic materials. I am also aware of the use of asphaltic compounds for waterproofing and cementing purposes and of the application of heat treated lacquers and primers over all surfaces of ferrous metal sheets prior to applying coatings thereto.

I am also aware of the use of foil-metal coverings as variously applied in the arts.

Having thus described my invention, I claim:

1. As a new article of manufacture, a roofing or building element of the class

described having a molded body, a coating of hydrocarbon waterproofing substance applied thereto on the surface to be exposed when in use and closing the pores thereof, and a non-ferrous metal protective covering over said coating and adhering thereto to give to the element a metal surfacing, said covering of foil-like thickness to prevent deterioration of said coating and to afford a finish and contribute strength to the element.

2. As a new article of manufacture, a roof or building element of the class described having a body of porous tile material, a foil-like non-ferrous metal outer covering, and an intermediate layer of an asphaltic substance adhering to both said body and said covering.

3. As a new article of manufacture, a roof or building element of the class described having a body of porous tile material, a foil-like non-ferrous metal outer covering, and an intermediate layer of an asphaltic substance adhering to both said body and said covering, said covering extending over the face of said body and extending about the edges thereof.

4. As a new article of manufacture, a roof or building element of the class described having a body of porous tile material, a foil-like non-ferrous metal outer covering, and an intermediate layer of an asphaltic substance adhering to both said body and said covering, said coating and said covering extending over the face of said body and extending about the edges thereof.

5. As a new article of manufacture, a roof or building element of the class described having a body of porous tile material and having a covering or surfacing formed of sheet metal of foil-like thickness.

6. As a new article of manufacture, a roof or building element of the class described having a body of porous tile material and having a covering or surfacing formed of sheet metal of foil-like thickness extending over the outer surface thereof and turned over the edges of the body.

LOUIS LANE.